

UNITED STATES PATENT OFFICE  
2,512,255

## HYDRAULIC FLUIDS

Charles W. Montgomery and William I. Gilbert,  
Oakmont, and Robert E. Kline, Penn Township,  
Allegheny County, Pa., assignors to Gulf Re-  
search & Development Company, Pittsburgh,  
Pa., a corporation of Delaware

No Drawing. Application December 31, 1947,  
Serial No. 795,160

8 Claims. (Cl. 252—79)

1

This invention relates to hydraulic fluids, and more particularly to fluids for use in hydraulically operated apparatus, such as brake mechanisms, fluid flywheels, shock absorbers, control mechanisms and similar hydraulically operated equipment. Various fluids have been previously proposed for use in hydraulic systems as hydraulic power transmission media or the like. In a great number of the previously proposed fluids, there have been many disadvantages attendant to their use, such as corrosive and degrading effects of such fluids on metal or rubber parts of the hydraulic equipment, a tendency towards volatilization at operating temperatures, lack of sufficient lubricating properties, etc.

It is an object of this invention, therefore, to provide a hydraulic fluid which overcomes the disadvantages of many of the prior art materials. It is a further object of this invention to provide hydraulic fluids which have general utility under variable operating conditions.

These and other objects are accomplished by the present invention wherein we provide as a hydraulic fluid for hydraulic equipment a liquid comprising an ester of an alcohol and naphthenic acid.

Naphthenic acids occur in certain crude oils, notably those of the Gulf Coast regions, California, Roumania, and Venezuela. These materials may be recovered from the oils in various ways, as known in the art. For example, crude oils may be distilled over caustic soda or lime whereupon the soaps of the naphthenic acids are retained in the stills along with tar and asphaltic ingredients. The soaps may then be recovered from these materials by washing with water, but difficulties are encountered with emulsions. Nevertheless, by using alcohol in the extraction, emulsions can be avoided and the acids recovered. The lighter acids are distilled over along with the oil distillates, and the naphthenic acids are removed from these with caustic soda more readily than from the heavy still bottoms because they are not contaminated with large amounts of pitch and asphalt. In separating the acids from oils, one method is to wash the oils with dilute caustic soda, say 0.5 to 5%, at a temperature above about 300° F., ordinarily not exceeding 500° F., and under a high pressure sufficient at least to prevent evaporation of the water. Under these conditions the acids are neutralized and are removed in the aqueous liquor which separates cleanly from the oil while at the high temperatures. The oil does not dissolve in the aqueous liquor to any appreciable extent and if

2

the separation of the aqueous and oily layers is effected hot, there is little hydrolysis of the soaps, so that the acid is substantially completely removed from the oil. The acids can then be recovered by acidification of the soap solutions with a mineral acid, which releases the naphthenic acids. These are then decanted and may be used as such, or they may be further purified, for example, by reconversion to soaps and reacidification or by distillation or similar processes.

Another method for recovering the acids consists in agitating a kerosene or gas oil distillate containing naphthenic acids with aqueous caustic soda, say 6° Bé., in an amount sufficient to neutralize all of the acid. The mixture is then allowed to settle for about 1 hour and the lower or aqueous layer is pumped off. The aqueous layer is then acidified with mineral acid, for example, 98% sulphuric acid, and the naphthenic acid separates as an upper layer, which is drawn off and washed with water until free of mineral acid.

The products of these extractions, which are the well known naphthenic acids of commerce, are complex mixtures of acidic compounds containing at least one carboxyl grouping. No general chemical structure can as yet be given to this group of acids, since the structural analyses of only a few have so far been determined. Many of the compounds appear to be characterized by having in their molecular structure one or more relatively saturated hydrocarbon rings, hence these extracted products are considered to be naphthenic acids. It would seem that the higher molecular weight compounds contain polycyclic groupings.

Properties of a typical naphthenic acid derived from petroleum are shown in the following table:

| Analytical data for naphthenic acids used in<br>making hydraulic fluids |                          |
|-------------------------------------------------------------------------|--------------------------|
|                                                                         | Naphthenic acids GR-7072 |
| Gravity, °API                                                           | 14.1                     |
| Sp. gr./60° F.                                                          | 0.9718                   |
| Vis. at 100° F. SUS                                                     | 767                      |
| Color, NPA                                                              | 5 (dilute)               |
| Flash point, COC, °F                                                    | 255                      |
| Fire point, COC, °F                                                     | 325                      |
| Carbon residue, Conradson                                               | 0.46                     |
| Neut. No                                                                | 199                      |
| Sap. No                                                                 | 206                      |
| Ash, per cent                                                           | 0.01                     |
| Sulfur, per cent                                                        | 0.11                     |

| Percent Dist. | Distillation Data at— |              |
|---------------|-----------------------|--------------|
|               | 10 mm., °F.           | 760 mm., °F. |
| I. B. P.      | 130                   | 341          |
| 10            | 332                   | 592          |
| 50            | 401                   | 678          |
| 90            | 469                   | 761          |

In order to obtain the hydraulic fluids of our invention, the naphthenic acids as obtained above are esterified with an alcohol to produce substantially neutral esters. The esterification may be conveniently carried out by refluxing 2 moles of an alcohol with 1 mole of the naphthenic acid for

If desired, the esters obtained as indicated above may be treated with lime and an adsorbent such as fuller's earth in order to purify the crude product. For example, in one such treatment the crude esters are stirred with about 4% by weight of fuller's earth and about 4% by weight of lime at a temperature of 150 to 200° C., and then are filtered.

The naphthenic esters may be employed in accordance with our invention either as the entire esterification product of the alcohol and the naphthenic acids or as selected fractions obtained by fractional distillation.

Representative properties of some of the esters of this invention are shown in the following table:

| Naphthenic Acid Ester     | Cut No. | Boiling Point Range °C., (Corr. to 760 mm.) | °API | Sp. Gr. 60/60° F. | Viscosity at— |             | Viscosity Index | Pour Point, °F. |
|---------------------------|---------|---------------------------------------------|------|-------------------|---------------|-------------|-----------------|-----------------|
|                           |         |                                             |      |                   | 100° F. SUS   | 210° F. SUS |                 |                 |
| n-Octyl Naphthenate       | 1       | 359-380                                     | 23.1 | 0.9153            | 59.9          | 35.4        | 116             | -40             |
|                           | 2       | 380-399                                     | 22.9 | 0.9165            | 67.0          | 35.8        | 98              | -35             |
|                           | 3       | 399-410                                     | 22.7 | 0.9176            | 76.7          | 37.2        | 97              | -30             |
|                           | 4       | 410-422                                     | 22.2 | 0.9206            | 88.9          | 38.4        | 98              | -15             |
|                           | 5       | 422-431                                     | 22.3 | 0.9200            | 107           | 40.0        | 98              | 0               |
|                           | 6       | 431-433                                     | 21.5 | 0.9248            | 137           | 43.6        | 99              | +30             |
|                           | 1       | 350-424                                     | 27.6 | 0.8894            | 92.9          | 37.8        | 46              | +65             |
|                           | 2       | 424-429                                     | 27.5 | 0.8899            | 66.8          | 36.4        | 115             | +25             |
|                           | 3       | 429-442                                     | 26.6 | 0.8950            | 77.5          | 37.7        | 119             | +25             |
|                           | 4       | 442-450                                     | 25.4 | 0.9018            | 98.9          | 39.9        | 123             | +25             |
| Lauryl Naphthenate        | 5       | 450-458                                     | 25.6 | 0.9007            | 105           | 40.6        | 127             | +25             |
|                           | 6       | 458-480                                     | 24.9 | 0.9047            | 127           | 42.8        | 128             | +25             |
|                           | 7       | 480-490                                     | 24.6 | 0.9065            | 147           | 44.3        | 124             | +40             |
|                           | 8       | 490-504                                     | 24.8 | 0.9053            | 169           | 46.2        | 125             | +50             |
|                           | 1-8     | 350-504                                     | 25.8 | 0.8996            | 101           | 40.0        | 118             | +35             |
|                           | 1       | 254-368                                     | 22.6 | 0.9182            | 55.1          | 53.8        | 62              | -65             |
|                           | 2       | 368-383                                     | 21.2 | 0.9267            | 83.8          | 36.8        | 29              | -70             |
|                           | 3       | 383-390                                     | 21.2 | 0.9267            | 89.3          | 37.6        | 53              | -65             |
| 2-Ethyl Hexyl Naphthenate | 4       | 390-398                                     | 21.2 | 0.9267            | 96.3          | 38.3        | 60              | -65             |
|                           | 5       | 398-411                                     | 21.2 | 0.9267            | 106           | 39.0        | 59              | -65             |
|                           | 6       | 411-422                                     | 21.2 | 0.9267            | 125           | 40.0        | 58              | -65             |
|                           | 7       | 422-441                                     | 21.2 | 0.9267            | 152           | 42.3        | 71              | -60             |
|                           | 8       | 441-483                                     | 20.5 | 0.9309            | 238           | 47.1        | 74              | -35             |
|                           | 1-8     | 254-483                                     | 21.4 | 0.9254            | 101           | 38.6        | 54              | -65             |

from about 5 to 12 hours in the presence of a small amount of anhydrous hydrogen chloride which acts as a catalyst. During this period water is continuously removed from the reaction mixture until the theoretical amount of separated water indicates that the reaction is complete, at which point the reaction is stopped. The excess alcohol is then distilled from the crude product and the residue is recovered. If desired the residue may be further purified by distilling under vacuum. Other methods of esterification may be employed as will be understood in the art.

A wide variety of alcohols may be employed for the esterification. Preferably these alcohols should be monohydric alcohols containing up to 20 carbon atoms such as methyl, ethyl, propyl, butyl, amyl, hexyl, octyl, decyl, lauryl, myristyl, palmityl, eicosyl, isopropyl, 2-ethyl-hexyl, allyl, crotonyl, oleyl propargyl, cyclohexanol, methylcyclohexanol, amylcyclohexanol, phenylcyclohexanol, cyclohexyl cyclohexanol, benzyl alcohol, phenylethyl alcohol, benzhydrol, tri-phenyl carbinol, phenylpropyl alcohol, phenylbenzyl alcohol, naphthobenzyl alcohol, cinnamyl alcohol, furfuryl alcohol, and tetrahydrofurfuryl alcohol. However, polyhydric alcohols may also be employed, such as ethylene glycol, propylene glycol, di-ethylene glycol, glycerol, and erythritol. Mixtures of any of the above alcohols may also be employed, particularly the mixtures of alcohols obtained by the reduction of coconut oil fatty acids; the mixture of higher molecular weight alcohols obtained as a by-product in the synthesis of methanol from carbon monoxide and hydrogen; as well as the mixture of alcohols obtained as a by-product in the synthesis of hydrocarbons from carbon monoxide and hydrogen.

The esters of the naphthenic acids obtained as described hereinabove present a number of properties making them eminently suitable as hydraulic fluids. As seen from the above table they possess a relatively high specific gravity; this property is very advantageous especially in momentum actuated hydraulic systems such as fluid flywheels. Furthermore the esters possess low volatility which means that at normal operating temperatures there will be practically no loss due to evaporation and very little loss even at relatively high operating temperatures.

In addition to the above characteristics these esters are susceptible to the action of pour point depressants, and therefore can be made to have a very low pour point. For example, one per cent by weight of a known pour point depressant, such as the condensation products of chlorinated wax and phenol followed by further condensation of the reaction product with organic acids, as exemplified by Santopour B which comprises the wax aryl esters of aromatic acids, will reduce the pour point of the lauryl ester from +45° F. to -5° F. Other known pour point depressants such as the condensation products of chlorinated wax and naphthalene may also be employed. In brief, the naphthenic acid esters present an aggregation of properties in a single material which render them particularly suitable for general use as hydraulic fluids.

Although we have disclosed the use of the esters of the naphthenic acids as hydraulic fluids by themselves, diluents and/or solvents may be added to the ester to produce homogeneous hydraulic fluids. When a diluent is used it will ordinarily be present in an amount from about 5 to 50% by weight of the esters of the naphthenic

acids depending upon the particular requirements, such as whether a light or a heavy grade of fluid is required for a particular application. Although the esters of the naphthenic acids are soluble in a wide variety of solvents, it is preferred to use relatively non-volatile solvents, as diluents of the esters in our hydraulic fluids. Typical classes of solvents which may be employed as diluents are: (1) the glycol ethers including the monobutyl ether of ethylene glycol, the mono-ethyl ether of ethylene glycol, the methyl ether of ethylene glycol mono-acetate, the butyl ether of diethylene glycol and the diethyl ether of ethylene glycol; and (2) hydrocarbon solvents such as light lubricating oils, gas oils, kerosene and the like.

The hydraulic fluids of the present invention, whether comprising the esters of the naphthenic acids alone or in combination with a pour point depressant or diluent as described above may be used as fluid power and transmission media in any of the common hydraulic systems wherein power is transmitted from an actuatable element to an actuated element by means of a fluid, the most common form of such a system comprising a pair of variable volume chambers with connecting conduit means, the chambers and the conduit means being filled with a fluid hydraulic power transmission medium. The hydraulic fluids of the present invention may, of course, also be used in analogous equipment in which power transmission is not the primary purpose of design, as for example in power absorption systems such as damping mechanisms, shock absorbers and the like.

In the following claims the expression "naphthenic acids" is employed to connote the mixture of acids of that name currently obtained in the petroleum refining industry, as well as naph-

thenic acid or acids which are now being synthetically prepared.

What we claim is:

1. The process which comprises transmitting power by means of a liquid consisting essentially of an ester of an alcohol and naphthenic acids.
- 5 2. The process of claim 1, wherein the alcohol is a monohydric alcohol.
- 10 3. The process of claim 1, wherein the alcohol is a monohydric alcohol containing up to 20 carbon atoms.
- 15 4. The process of claim 1, wherein the alcohol is lauryl alcohol.
- 15 5. The process of claim 1, wherein the alcohol is n-octyl alcohol.
- 20 6. The process of claim 1, wherein the alcohol is 2-ethyl-hexyl alcohol.
7. The process of claim 1, wherein the liquid contains additionally a pour point depressant.
- 20 8. The process of claim 1, wherein the liquid contains additionally from about 5 to 50 per cent by weight of a relatively non-volatile liquid diluent.

CHARLES W. MONTGOMERY.

WILLIAM I. GILBERT.

ROBERT E. KLINE.

#### REFERENCES CITED

The following references are of record in the file of this patent:

#### UNITED STATES PATENTS

| Number       | Name         | Date          |
|--------------|--------------|---------------|
| 2,033,853    | Sherbino     | Mar. 10, 1936 |
| 35 2,048,466 | Reiff et al. | July 21, 1936 |
| 2,091,627    | Bruson       | Aug. 31, 1937 |
| 2,147,545    | Reiff        | Feb. 14, 1939 |
| 2,195,131    | Kapp et al.  | Mar. 26, 1940 |
| 2,250,265    | Kapp et al.  | July 22, 1941 |
| 40 2,417,088 | Prutton      | Mar. 11, 1947 |